

Jan. 23, 1934.

E. ORIOLI

1,944,299

PROCESS AND APPARATUS FOR DRY SPINNING ARTIFICIAL SILK

Filed April 5, 1930

2 Sheets-Sheet 1

Fig. 1.



Fig. 3.



Fig. 5.



Fig. 2.



Fig. 4.



Fig. 6.



INVENTOR

Ernesto Orioli

BY  
Gifford, Seel & Burgess

ATTORNEYS

Jan. 23, 1934.

E. ORIOLI

1,944,299

PROCESS AND APPARATUS FOR DRY SPINNING ARTIFICIAL SILK

Filed April 5, 1930

2 Sheets-Sheet 2

Fig. 7.



Fig. 8.



Fig. 9.



Fig. 10.



INVENTOR

Ernesto Orioli

BY

Gifford, Seal & Burgess

ATTORNEYS

## UNITED STATES PATENT OFFICE

1,944,299

PROCESS AND APPARATUS FOR DRY  
SPINNING ARTIFICIAL SILKErnesto Orioli, Milan, Italy, assignor to Ruth-  
Aldo Company, Inc., a corporation of New  
YorkApplication April 5, 1930, Serial No. 442,027, and  
in Italy November 11, 1929

11 Claims. (Cl. 18—8)

This invention relates to a process and apparatus for dry spinning artificial silk, which is often referred to as "rayon." By this invention, filaments are produced in such a manner that the objectionable sparkling effects of the same are greatly minimized or entirely overcome.

It is well known that in the dry spinning of cellulose esters or ethers elementary filaments are easily obtained having a flat cross-section and smooth edges or in cross-section somewhat like a dumb-bell. Such flossy filaments in the form of a ribbon produce in yarns special sparkling effects which greatly reduce the possibility of employing them.

To avoid this defect, different proceedings have been proposed, in order to obtain elementary filaments having star-like cross-sections.

I have now found that the cross-section of the collodion jet issuing from the spinning nozzle can be favorably influenced by a hot current of gas and vapors taken from the spinning cell itself.

In my invention, a pipe may be located in the spinning cell or near the cell. This pipe is open at both ends and connects the space around the spinning nozzle with the lower part of the cell. This pipe may be heated internally by an electric heater or by an interior pipe of a smaller diameter in which a heating medium circulates or it may be heated externally by a jacket. The inside temperature of the pipe is higher than the average temperature of the spinning cell, so that a rising gas current is produced in the inside of the pipe and this current strikes the collodion jets issuing out of the spinning nozzle, creating favorable conditions of evaporation of the solvent in order to cause the desirable cross-section of the filaments to be obtained.

In the application of Raymond A. J. Thenoz, Serial No. 423,166, filed January 24, 1930, there was described a process and apparatus for producing a dull luster rayon by causing a shifting or movement of gases at an angle to the path of the jets adjacent the spinneret before the filaments harden, this shifting or movement of the gases being produced by a fan or the like. By the present invention, a shifting or movement of gases which strike the filaments at an angle is produced by heating the gases in a particular way and permitting them to rise.

The invention will be understood from the description in connection with the accompanying drawings, in which Fig. 1 is a vertical section through a spinning cell or chamber; Fig. 2 is a section along the line 2—2 of Fig. 1; Figs. 3 and

5 are vertical sections through modifications of the spinning cell; Figs. 4 and 6 are sections along the line 4—4 of Fig. 3 and 6—6 of Fig. 5, respectively; Fig. 7 is a vertical section showing a double spinning cell; Fig. 8 is a vertical section between the cells taken at right angles to Fig. 7; Fig. 9 is a section along the line 9—9 of Fig. 7, and Fig. 10 is a section along the line 10—10 of Fig. 7.

In the drawings, reference character 1 indicates a spinning cell or chamber having a jacket 2 surrounding the same, so that it can be heated in the well known manner by passing a heating fluid through the jacket. An inlet 3 is provided near the bottom of the cell for the introduction of air or gas to remove the solvent from the filament and leave a hard filament, and the outlet for the air or gas is shown at 4 near the upper end of the cell. Openings 5 may be provided as indicated, with windows for inspection of the interior of the cell.

A spinneret with its supporting pipe 6 which is of the well known type, is located at the upper end of the cell for extruding or squirting filaments into the cell, and the cone 7 is provided at the bottom for removing the filaments.

A vertically extending pipe 8 having its lower end open and having an outlet 9 near the top is located in the cell 1 to one side of the center line, so that the outlet 9 will be near the outlet of the spinneret 6. A heating coil 10, which may be an electrical or other sort of heater, is located in the pipe 8, so that the air or gas inside of this pipe will be heated and rise to strike the filaments at an angle as they issue from the spinneret.

In the other modifications, the parts that are common to the embodiment of the cell already described are referred to by the same reference characters and the description will not be repeated.

In the modification shown in Figs. 3 and 4, the vertically extending pipe 11 through which the hot air or gas rises is located outside of the chamber or cell 1 with its lower end 12 extending through the wall of this cell near the bottom. The upper end of the pipe 11 has an outlet 13 also extending through the wall of the cell 1 close to the spinneret 6. The pipe 11 is heated by a smaller pipe 14 extending a portion of the way therethrough with its lower end 15 extending through the side of the pipe 11 and through the wall of the jacket 2, near the lower end thereof. A pipe 16 leads away from the upper end of the jacket. A heating fluid is passed through the

pipe 14 for heating the air in the pipe 11 and this heating fluid then passes through the jacket 2 and out through the pipe 16.

- 6 In the modification shown in Figs. 5 and 6, the lower end 18 of the vertically extending pipe 17 extends some distance into the interior of the chamber 1 and the outlet 19 from the pipe 17 also extends some distance into this chamber into proximity to the lower end of the spinneret 6.
- 10 A heating pipe 20 extends some distance along the inside of the pipe 17 and thence into the jacket 2, as indicated at 21. An outlet pipe 22 for the heating fluid extends from the upper portion of the jacket 2.

- 15 In the modification shown in Figs. 7 to 10, two cells or chambers are shown spaced apart and having their walls connected by a chamber or housing made up of plates 23. An inlet 24 is provided near the lower end of each cell into the lower portion of the housing, and corresponding outlets 25 are provided at the upper portion, so that the hot air or gases rising in this housing impinge against the sides of the filaments as they emerge from the spinnerets 6. A U-shaped pipe 26 for the hot fluid for heating the chamber between the cells extends longitudinally through the chamber.

30 In each one of the illustrated devices, air or gas is heated to a temperature above the temperature of the main body of the air or gas in the cell so as to produce an upwardly rising jet or current of air or gas that strikes against the sides of the filaments, thus producing the desired effect, both because of the physical contact of 35 the air or gas against the filaments and also because this air or gas is at a higher temperature.

35 Subjecting the filaments issuing from the spinnerets to the hot lateral air currents, as described above, causes them to assume irregular shapes 40 in cross-section during the hardening thereof. The lateral current or deflection of gas so affects the evaporation of the solvent from the filaments during the formative and hardening steps that, instead of contracting regularly and uniformly 45 to form round filaments or filaments with a dumbbell cross-section, they contract irregularly to form filaments of cross-sections such that the light is partially reflected, but is largely diffused by the surfaces of the filaments, with the result 50 that the yarn and fabrics produced from such filaments do not have the high luster of ordinary rayon, but instead have a dull luster, which is so much desired in present day fabrics of this sort.

55 The invention is applicable to the ordinary spinning cell, to which a vertically disposed pipe and heating means may be added. The temperatures used may be substantially the same as in the ordinary cell and the gas employed in the 60 cell, as well as the quality of the solutions employed in forming the filament, can remain unchanged.

I claim:

- 65 1. In the manufacture of rayon the process for distorting the rayon filament surface which comprises extruding a spinning solution as a filament into a solvent-evaporating gas at a suitable temperature and subjecting the filament

80 movement in the extrusion zone to lateral pressure of a gas at a higher temperature than the main body of evaporating gas in said zone, said lateral pressure being unequal around the periphery of the filament in said zone.

85 2. In the manufacture of rayon the process for distorting the rayon filament surface which comprises extruding a spinning solution as a filament into a solvent-evaporating gas at a suitable temperature in a zone secluded from the outside air and introducing laterally into said zone along a restricted part of the periphery thereof a transverse current of solvent-evaporating gas heated to a higher temperature than the main body of evaporating gas in said zone.

90 3. In the manufacture of rayon the process for distorting the rayon filament which comprises extruding a spinning solution as a filament into a solvent-evaporating gas at a suitable temperature and directing against a side of the filament while in plastic condition a current of gas at a higher temperature than the main body of evaporating gas.

95 4. In the manufacture of rayon the process for distorting the rayon filament which comprises extruding a spinning solution as a filament into a solvent-evaporating gas heated to a suitable temperature and subjecting the filament while plastic to the lateral impact of a unidirectional current of solvent-evaporating gas heated to a higher temperature than the main body of evaporating gas.

100 5. In the manufacture of rayon the process for distorting the rayon filament surface which comprises extruding a spinning solution as a filament into a solvent-evaporating gas, producing an upward current of heated gas by heating such gas in a vertically extending passage and directing said current laterally against one side of the filament.

105 6. Apparatus for dry spinning rayon filaments including a spinning cell, a spinneret, a passage for heated gas and a nozzle at the end of said passage positioned at one side of the cell to direct a current of said gas across the cell against one side of the filament while the latter is in a plastic state.

110 7. Apparatus for dry spinning rayon filaments including a spinning cell, a spinneret, an upwardly extending passage for heated gas having an outlet positioned at one side of the cell for projecting heated gas against a side of the filament while the latter is in a plastic state, and means for heating gas in the passage.

115 8. Apparatus as set forth in claim 7 in which the heating means extends into the passage.

9. Apparatus as set forth in claim 7 in which the inlet to said passage opens into the cell.

10. Apparatus as set forth in claim 7 in which the passage is located within the cell.

135 11. Apparatus for dry spinning rayon filaments including a spinning cell, a spinneret, a passage for heated solvent-evaporating gas having an outlet in the cell positioned to direct a current of said gas across the path of the filament while the latter is in a plastic state, and common heating means for said passage and cell.

ERNESTO ORIOLI.